

No. 664,659.

Patented Dec. 25, 1900.

P. M. MATTHEW.

CORSET SHIELD.

(Application filed Oct. 21, 1899.)

(No Model.)

*Fig. 1.*



*Fig. 2.*



*Fig. 3.*



WITNESSES:

*L.C. Hilly.*  
*Walter Allen*

Patrick M. Matthew  
BY *Knights Bros*  
Attorneys

# UNITED STATES PATENT OFFICE.

PATRICK MILLAR MATTHEW, OF EDINBURGH, SCOTLAND.

## CORSET-SHIELD.

SPECIFICATION forming part of Letters Patent No. 664,659, dated December 25, 1900.

Application filed October 21, 1899. Serial No. 734,287. (No model.)

*To all whom it may concern:*

Be it known that I, PATRICK MILLAR MATTHEW, a subject of the Queen of the United Kingdom of Great Britain and Ireland, residing at Victoria India Rubber Mills, Leith Walk, Edinburgh, in the county of Mid-Lothian, Scotland, have invented new and useful Improvements in Corset-Shields, of which the following is a specification.

My invention, as hereinafter described, relates to the production of the flexible stay-pieces or supports (commonly known as "corset-shields") which are applied to the inner surfaces of corsets at each side at the points where, curving to fit the waist of the wearer, the steels or bones of the corsets are liable to fracture from the movements of the body. The object of my invention is to provide shields which shall be so flexible and elastic as to adapt themselves to the curves of the body with perfect ease and comfort to the wearer and which shall at the same time be sufficiently rigid to afford the support necessary to prevent the fracture of the steels or bones of the corset by the movements of the body. They may either be fitted to corsets in the course of manufacture of the latter or they may afterward be attached in a suitable manner to the finished corsets. They may also be applied to corsets in which the steels or bones have already become fractured at the points above indicated, and when so applied they will effectually prevent injury to the person or clothing of the wearer from the broken ends of the steels or bones.

The shields which are the subject of this invention consist, primarily, of thin sheets of india-rubber, compounded and vulcanized in such a manner as to combine the necessary rigidity, flexibility, and elasticity above referred to. The form and size of the shields may be varied according to the size of the corsets to which they are to be applied or other circumstances. For general purposes I have found an elliptical form most suitable, as illustrated in the accompanying drawings, in which—

Figure 1 is a plan view of my improved corset-shield, consisting of a combined rubber and fiber sheet. Fig. 2 is a plan view of the same provided with fabric covering. Fig. 3 is a central longitudinal section thereof.

In carrying out my invention I first prepare the rubber by adding thereto a proportion of fibrous material *a*, such as cotton or jute, 55 which I reduce to a fine state of division and closely incorporate with the rubber by means of such grinding and mixing machinery as is commonly employed in rubber factories for analogous purposes. I have found that twenty-four parts, by weight, of rubber to 60 twelve parts, by weight, of fiber are suitable proportions. To this combined rubber and fiber compound I then add the necessary vulcanizing ingredients (preferably litharge and 65 sulfur) in such proportions as will render the rubber sufficiently rigid and flexible after having been subsequently submitted to the process of vulcanization. I have found that eight parts, by weight, of litharge and one 70 part, by weight, of sulfur to twenty-four parts, by weight, of rubber are suitable proportions for producing the required result. The rubber and fiber compound thus prepared is then formed into sheets of the required thickness 75 by means of the ordinary process of calendering rubber sheets. The thickness of the sheets may be varied according to the particular amount of rigidity which is desired; but for general purposes I find that about one-sixteenth of an inch is ample. The sheets are then vulcanized by any suitable method; but I prefer to employ the ordinary hot press, in which the rubber is vulcanized under pressure between two metal plates heated by 85 steam to the required temperature.

The shields *A* may either be cut from the sheet after vulcanization or prior to it. In the latter case they must be vulcanized after being cut, and preferably so by the hot press, 90 as above described.

The combined rubber and fiber sheet prepared by the method above described is capable of being stretched in one direction only—that is to say, on its width or at right angles 95 to the direction in which it leaves the calender—and in cutting the shields from the sheet it is absolutely necessary that its horizontal axis should lie in the direction in which the rubber can be stretched. This permits 100 the shield when being drawn into contact with the body of the wearer to expand along the upper or lower portions of its periphery, as indicated by the double-headed arrow *B*, and

thus to adapt itself with absolute accuracy to the double curvature of the body at the waist of the wearer.

For the sake of appearance, as well as for the purpose of giving additional strength to the shields, I prefer to cover them on both sides by a cotton or other fabric C of suitable texture. This fabric I prepare by coating it on one side with an adhesive solution of India-rubber capable of being vulcanized. I then attach the fabric by means of pressure to both sides of the rubber sheet prior to the vulcanization of the latter, or, having cut the prepared fabric into portions of the necessary size and shape, I attach them by similar means to the shields which have been cut from the unvulcanized rubber sheet, as above stated. In the latter case, being that shown in the drawings, the portions of the fabric may be cut somewhat larger than the rubber shield, so that they will overlap the edge of the latter, and their two adhesive surfaces coming in contact will form a flange c around the shield. In either case the material is then vulcanized, as before described.

In order that the expansion of the shields at the proper parts may not be interfered with by the overlying fabric, it is necessary that the latter be made or cut in such a manner that it will possess the necessary amount of elasticity in the required direction—that is to say, a fabric which is not elastic in make should be cut on the bias, as indicated by the lines on Fig. 2 of the drawings.

For the purpose of enabling the shields to be stitched to the corset small holes may be punched through the rubber at suitable intervals and fitted with eyelets D, and additional holes may similarly be formed, if desired, for purposes of ventilation.

My invention depends in part upon the discovery that this principle can be utilized with especially advantageous effect in the construction of corset-shields by cutting from such composite fabric sheets of the proper elliptical shape to form corset-shields with the fibers or threads in the composite sheet running crosswise in the elliptical sheet; so that when said shields are made up and applied to corsets in the usual position with the major axis of the ellipse in horizontal position the tensile strength of the sheet transversely of its length will afford the necessary strength to the shield to prevent breaking by vertical tension, in which direction the shields are subject to the most severe tensile strain, while the flexibility of the threads or fibers permits the shield to bend forward in a vertical plane, and at the same time the parallel vertical disposition of the threads in the composite sheet affords great elasticity thereto in a horizontal direction or lengthwise of the sheet or shield, and this elasticity permits the

shield to curve freely backward in a horizontal plane. By the flexibility of the threads I provide for the forward vertical curvature, and by their vertical disposition I provide the requisite tensile strength to prevent breaking and leave the rubber free to stretch in a horizontal direction. The shield is thus enabled to curve in both a vertical and horizontal direction forward and backward, respectively, as required to conform to the curvature of the human waist without undue strain or violence to the material. I furthermore provide the sheet or shield with a covering of woven fabric cut on the bias, so as to be elastic in both directions, and thus not interfere with the freedom of the curvature in two directions at once, as above described.

I lay no claim, broadly, to the fabric covering, as such covering is only for the purpose of appearance and to keep the fibrous rubber from coming into direct contact with the wearer. The said cover in no way assists the required peculiar properties of the fibrous-rubber compound, these said peculiar properties being attained, as hereinbefore described, by the peculiar process of manufacture and by the particular method of cutting from the sheet.

Having thus described my invention, the following is what I claim as new therein and desire to secure by Letters Patent:

1. A corset-shield comprising a thin combined rubber and fiber sheet in which the fibers are thoroughly mixed with the rubber, extend vertically crosswise of the sheet and overlap so as to break joint whereby the tensile strength of the fibers prevents breaking by vertical strain while their flexibility permits the bending of the sheet in a vertical plane; and whereby the curvature of the sheet in a horizontal plane is permitted by the elasticity of the sheet in that direction.

2. A corset-shield comprising a thin combined rubber and fiber sheet of customary elliptical form, having the fibers disposed crosswise of the sheet so as to be in vertical position when in use and overlapping so as to break joint and a fabric covering cut on the bias, and secured to the sheet, as explained.

3. A corset-shield comprising a thin combined rubber and fiber sheet of elliptical shape having the fibers disposed crosswise of the sheet so as to assume a vertical position when in use and overlapping so as to break joint, and fabric coverings cut on the bias, and each having an adhesive coating whereby they are applied under pressure to the thin sheet so as to permit the thin sheet to yield in the manner explained.

PATRICK MILLAR MATTHEW

Witnesses:

FRANCIS ROBERT MILNE,  
COLIN ROSS CROMBIE.